

# United States Patent [19]

Bowes et al.

[11] Patent Number: 4,876,411

[45] Date of Patent: Oct. 24, 1989

[54] MODIFIED CRYSTALLINE ALUMINOSILICATE ZEOLITE CATALYST AND ITS USE IN THE PRODUCTION OF LUBES OF HIGH VISCOSITY INDEX

[75] Inventors: Emmerson Bowes, Hopewell; Clarence D. Chang, Princeton; Scott Han, Lawrenceville; David S. Shihabi, Pennington, all of N.J.

[73] Assignee: Mobil Oil Corporation, New York, N.Y.

[21] Appl. No.: 27,034

[22] Filed: Mar. 19, 1987

## Related U.S. Application Data

[63] Continuation of Ser. No. 815,956, Jan. 3, 1986, abandoned.

[51] Int. Cl.<sup>4</sup> C07C 2/02

[52] U.S. Cl. 585/533; 502/71; 502/77; 502/85; 502/86

[58] Field of Search 208/18; 583/502, 533; 502/71, 77, 86, 85

## References Cited

### U.S. PATENT DOCUMENTS

- |           |         |                 |         |
|-----------|---------|-----------------|---------|
| 3,322,848 | 5/1967  | Garwood et al.  | 585/533 |
| 4,413,153 | 11/1983 | Garwood et al.  | 585/408 |
| 4,512,961 | 4/1985  | Scherzer et al. | 502/79  |
| 4,531,014 | 7/1985  | Gregory et al.  | 585/533 |
| 4,547,613 | 10/1985 | Garwood et al.  | 585/408 |
| 4,560,542 | 12/1985 | Robson          | 502/60  |
| 4,665,250 | 5/1987  | Chu et al.      | 585/407 |
| 4,754,906 | 6/1988  | Chang et al.    | 585/533 |
| 4,788,374 | 11/1988 | Chu et al.      | 585/533 |
| 4,788,375 | 11/1988 | Garwood et al.  | 585/533 |

## FOREIGN PATENT DOCUMENTS

- |         |         |                    |         |
|---------|---------|--------------------|---------|
| 0095304 | 11/1983 | European Pat. Off. | 423/328 |
| 0095305 | 11/1983 | European Pat. Off. | 502/79  |
| 0142313 | 5/1985  | European Pat. Off. | 502/85  |

## OTHER PUBLICATIONS

Kerr, "Chemistry of Crystalline Aluminosilicates V. Preparation of Aluminum-Deficient Faujasites", *The Journal of Physical Chemistry*, vol. 72, No. 7, Jul. 1968, pp. 2594-2596.

Dwyer et al., "The Surface Composition of Dealuminated Zeolites", *J.C.S. Chem. Comm.*, 1981, pp. 422-424.

Gross et al., "Surface Composition of Dealuminated Y Zeolites Studied by X-Ray Photoelectron Spectroscopy", *Zeolites*, 1984, vol. 4, Jan., pp. 25-29.

Primary Examiner—Anthony McFarlane  
Attorney, Agent, or Firm—A. J. McKillop; Charles J. Speciale; Edward F. Kenehan, Jr.

## ABSTRACT

The present invention provides a process for modifying a crystalline aluminosilicate zeolite having a Constraint Index of from about to about 12 which comprises:

- steaming the as synthesized crystalline aluminosilicate zeolite containing organic template material to decompose at least a portion of said template material and to extract zeolitic aluminum; and,
- contacting the zeolite resulting from step (a) in the ammonium, alkali metal or hydrogen form with a dealuminizing agent which forms a water-soluble complex with aluminum to remove a further quantity of zeolitic aluminum therefrom wherein said treated catalyst is employed in the making of lube oil from olefins.

9 Claims, No Drawings

MODIFIED CRYSTALLINE ALUMINOSILICATE  
ZEOLITE CATALYST AND ITS USE IN THE  
PRODUCTION OF LUBES OF HIGH VISCOSITY  
INDEX

This is a continuation of copending application Ser. No. 815,956, filed on Jan. 3, 1986, now abandoned.

BACKGROUND OF THE INVENTION

The present invention relates to modification of a crystalline aluminosilicate zeolite catalyst having a Constraint Index of from about 10 to about 12, e.g., ZSM-5, to reduce external acid sites thereon and a process for preparing high viscosity index (VI) lubes employing the modified catalyst.

Zeolitic materials, both natural and synthetic, have been demonstrated in the past to have catalytic properties for various types of hydrocarbon conversion. Certain zeolitic materials are ordered, porous crystalline aluminosilicates having a definite crystalline structure as determined by X-ray diffraction within which there are a number of smaller cavities which may be interconnected by a number of still smaller channels or pores. These cavities and pores are uniform in size within a specific zeolitic material. Since the dimensions of these pores are such as to accept for absorption molecules of certain dimensions while rejecting those of larger dimensions, these materials have come to be known as "molecular sieves" and are utilized in a variety of ways to take advantage of these properties.

Such molecular sieves, both natural and synthetic, include a wide variety of positive ion-containing crystalline aluminosilicates. These aluminosilicates can be described as a rigid three-dimensional framework of  $\text{SiO}_4$  and  $\text{AlO}_4$  in which the tetrahedra are cross-linked by the sharing of oxygen atoms whereby the ratio of the total aluminum and silicon atoms to oxygen atoms is 1:2. The electrovalence of the tetrahedra containing aluminum is balanced by the inclusion in the crystal of a cation, for example an alkali metal or an alkaline earth metal cation. This can be expressed wherein the ratio of aluminum to the number of various cations, such as  $\text{Ca}/2$ ,  $\text{Sr}/2$ ,  $\text{Na}$ ,  $\text{K}$  or  $\text{Li}$ , is equal to unity. One type of cation may be exchanged either entirely or partially with another type of cation utilizing ion exchange techniques in a conventional manner. By means of such cation exchange, it has been possible to vary the properties of a given aluminosilicate by suitable selection of the cation. The spaces between the tetrahedra are occupied by molecules of water prior to dehydration.

Prior art techniques have resulted in the formation of a great variety of synthetic zeolites. The zeolites have come to be designated by letter or other convenient symbols, as illustrated by zeolite Z (U.S. Pat. No. 2,882,243), zeolite X (U.S. Pat. No. 2,882,244), zeolite Y (U.S. Pat. No. 3,130,007), zeolite ZK-5 (U.S. Pat. No. 3,247,195), zeolite Beta, (U.S. Pat. No. 3,308,069), zeolite ZK-4 (U.S. Pat. No. 3,314,752), zeolite ZSM-5 (U.S. Pat. No. 3,702,886), zeolite ZSM-11 (U.S. Pat. No. 3,709,979), zeolite ZSM-12 (U.S. Pat. No. 3,832,449), zeolite ZSM-20 (U.S. Pat. No. 3,972,983), ZSM-35 (U.S. Pat. No. 4,016,245), ZSM-38 (U.S. Pat. No. 4,046,859) and zeolite ZSM-23 (U.S. Pat. No. 4,076,842), merely to name a few.

U.S. Pat. No. 4,461,845 teaches a method for reactivating a steam-deactivated catalyst comprising a zeolite having a silicon/aluminum atomic ratio of at least 2.

The method involves contact with an aluminum compound at elevated temperature, followed by contact with an aqueous acid solution. U.S. Pat. No. 4,477,582 teaches a method for reactivating a steam-deactivated catalyst comprising a zeolite having a silicon/aluminum ratio of at least 3.5. The method of this patent involves contact with an alkali, alkaline earth or transition metal salt solution followed by contact with an aqueous ammonium ion solution.

In accordance with U.S. Pat. No. 4,503,023, aluminum from  $\text{AlO}_4$ -tetrahedra of zeolites is extracted and substituted with silicon to form zeolite compositions having higher  $\text{SiO}_2/\text{Al}_2\text{O}_3$ . The preparative procedure involves contact of the starting zeolite having an  $\text{SiO}_2/\text{Al}_2\text{O}_3$  molar ratio of about 3 or greater with an aqueous solution of a fluorosilicate salt using controlled proportions and temperature and pH conditions which are intended to avoid aluminum extraction without silicon substitution. The fluorosilicate salt serves as the aluminum extractant and as the source of extraneous silicon which is inserted into the zeolite structure in place of the extracted aluminum.

U.S. Pat. No. 4,427,790 describes a process for improving the activity of crystalline zeolite in which the zeolite in the "as synthesized" form or following ion-exchange is reacted with a compound having a complex fluoranion.

The use of chelating agents to remove framework and non-framework aluminum from faujasite materials is shown by G. T. Kerr, "Chemistry of Crystalline Aluminosilicates. V. Preparation of Aluminum Deficient Faujasites", *J. Phys. Chem.* (1968) 72 (7) 2594; T. Gross et al., "Surface Composition of Dealuminized Y Zeolites Studied by X-Ray Photoelectron Spectroscopy", *Zeolites* (1984) 4, 25; and J. Dwyer et al., "The Surface Composition of Dealuminized Zeolites", *J. Chem. Soc., Chem. Comm.* (1981) 42.

Other references teaching removal of aluminum from zeolites include U.S. Pat. No. 3,442,795, and U.K. Pat. No. 1,058,188 (hydrolysis and removal of aluminum by chelation); U.K. Pat. No. 1,061,847 (acid extraction of aluminum); U.S. Pat. No. 3,493,519 (aluminum removal by steaming and chelation); U.S. Pat. No. 3,591,488 (aluminum removal by steaming); U.S. Pat. No. 4,273,753 (dealumination by silicon halides and oxyhalides); U.S. Pat. No. 3,691,099 (aluminum extraction with acid); U.S. Pat. No. 4,093,560 (dealumination by treatment with salts); U.S. Pat. No. 3,937,791 (aluminum removal with Cr(III) solutions); U.S. Pat. No. 3,506,400 (steaming followed by chelation); U.S. Pat. No. 3,640,681 (extraction of aluminum with acetylacetone followed by dehydroxylation); U.S. Pat. No. 3,836,561 (removal of aluminum with acid); German Pat. No. 2,510,740 (treatment of zeolite with chlorine or chlorine-containing gases at high temperatures); Netherlands Pat. No. 7,604,264 (acid extraction), Japan Pat. No. 53/101,003 (treatment with EDTA or other materials to remove aluminum) and *J. Catalysis*, 54, 295 (1978) (hydrothermal treatment followed by acid extraction).

The use of ZSM-5 type zeolites in the conversion of olefins to provide lubricating oils is known, inter alia, from U.S. Pat. Nos. 4,520,221 and 4,524,232. In the former, surface acidity of a ZSM-5 zeolite catalyst is neutralized by treating with a sterically hindered base such as 2,6-di-tert-butylpyridine. Employing the base-modified catalyst, propylene was converted to lubes with a 60 VI number increase over a lube oil prepared with the unmodified catalyst. The base must be added

continuously during the conversion process. At high reaction severities, the base will react with the feed, a practical limitation on the use of such a catalyst.

#### SUMMARY OF THE INVENTION

In accordance with the present invention, the surface acidity of a crystalline aluminosilicate zeolite catalyst having a Constraint Index of from about 1 to 12 is reduced to provide a modified zeolite having enhanced catalytic activity for a variety of hydrocarbon conversions and, in particular, for the oligomerization of olefin to provide lubes of high viscosity index.

Thus, the present invention provides a process for modifying a crystalline aluminosilicate zeolite having a Constraint Index of from about 1 to about 12 which comprises:

(a) steaming the as synthesized crystalline aluminosilicate zeolite containing organic template material to decompose at least a portion of said template material and to extract zeolitic aluminum; and,

(b) contacting the zeolite resulting from step (a) in the ammonium, alkali metal or hydrogen form with a dealuminizing agent which forms a water-soluble complex with aluminum to remove a further quantity of zeolitic aluminum therefrom.

The foregoing treatment results in the reduction of acid sites on the zeolite essentially without affecting its internal structure. As a result, the incidence of undesirable side reactions tending to occur on the surface of the untreated catalyst and which result in lower product yield and/or inferior product characteristics is significantly lessened.

#### DESCRIPTION OF THE PREFERRED EMBODIMENTS

The crystalline zeolites which are modified in accordance with this invention are members of a novel class of zeolitic materials which exhibit unusual properties. Although these zeolites have unusually low alumina contents, i.e., high silica to alumina mole ratios, they are very active even when the silica to alumina mole ratio exceeds 30. The activity is surprising since catalytic activity is generally attributed to framework aluminum atoms and/or cations associated with these aluminum atoms. These zeolites retain their crystallinity for long periods in spite of the presence of steam at high temperature which induces irreversible collapse of the framework of other zeolites, e.g., of the X and A type. Furthermore, carbonaceous deposits, when formed, may be removed by burning at higher than usual temperatures to restore activity. These zeolites, used as catalysts, generally have low coke-forming activity and therefore are conducive to long times on stream between regenerations by burning carbonaceous deposits with an oxygen-containing gas such as air.

An important characteristic of the crystal structure of this novel class of zeolites is that it provides a selective constrained access to, and egress from, the intracrystalline free space by virtue of having an effective pore size intermediate between the small pore Linde A and the large pore Linde X, i.e., the pore windows of the structure are of about a size such as would be provided by 10-membered rings of silicon atoms interconnected by oxygen atoms. It is to be understood, of course, that these rings are those formed by the regular disposition of the tetrahedra making up the anionic framework of the crystalline zeolite, the oxygen atoms themselves

being bonded to the silicon (or aluminum, etc.) atoms at the centers of the tetrahedra.

The silica to alumina mole ratio referred to may be determined by conventional analysis. This ratio is meant to represent, as closely as possible, the ratio in the rigid anionic framework of the zeolite crystal and to exclude aluminum in the binder or in cationic or other form within the channels. Although zeolites with silica to alumina mole ratios of at least 12 are useful, it is preferred to use zeolites having substantially higher silica/alumina ratios, e.g., 70 and above.

The novel class of zeolites, after activation, acquire an intracrystalline sorption capacity for normal hexane which is greater than that for water, i.e. they exhibit "hydrophobic" properties. This hydrophobic character can be used to advantage in some applications.

The novel class of zeolites to undergo modification as more fully described, infra, have an effective pore size such as to freely sorb normal hexane. In addition, the structure must provide constrained access to larger molecules. It is sometimes possible to judge from a known crystal structure whether such constrained access exists. For example, if the only pore windows in a crystal are formed by 8-membered rings of silicon and aluminum atoms, then access by molecules of larger cross-section than normal hexane is excluded and the zeolite is not of the desired type. Windows of 10-membered rings are preferred, although in some instances excessive puckering of the rings or pore blockage may render these zeolites ineffective.

Although 12-membered rings in theory would not offer sufficient constraint to produce advantageous conversions, it is noted that the puckered 12-ring structure of TMA offretite does show some constrained access. Other 12-ring structures may exist which may be operative for other reasons and, therefore, it is not the present intention to entirely judge the usefulness of a particular zeolite solely from theoretical structural considerations.

Rather than attempt to judge from crystal structure whether or not a zeolite possesses the necessary constrained access to molecules of larger cross-section than that of normal paraffins, a simple determination of the "Constraint Index" as herein defined may be made by passing continuously a mixture of an equal weight of normal hexane and 3-methylpentane over a sample of zeolite at atmospheric pressure according to the following procedure. A sample of the zeolite, in the form of pellets or extrudate, is crushed to a particle size about that of coarse sand and mounted in a glass tube. Prior to testing, the zeolite is treated with a stream of air at 540° C. for at least 15 minutes. The zeolite is then flushed with helium and the temperature is adjusted between 290° C. and 510° C. to give an overall conversion of between 10% and 60%. The mixture of hydrocarbons is passed at 1 liquid hourly space velocity (i.e., 1 volume of liquid hydrocarbon per volume of zeolite per hour) over the zeolite with a helium dilution to give a helium to (total) hydrocarbon mole ratio of 4:1. After 20 minutes on stream, a sample of the effluent is taken and analyzed, most conveniently by gas chromatography, to determine the fraction remaining unchanged for each of the two hydrocarbons.

While the above experimental procedure will enable one to achieve the desired overall conversion of 10 to 60% for most zeolite samples and represents preferred conditions, it may occasionally be necessary to use somewhat more severe conditions for samples of very

low activity, such as those having an exceptionally high silica to alumina mole ratio. In those instances, a temperature of up to about 540° C. and a liquid hourly space velocity of less than one, such as 0.1 or less, can be employed in order to achieve a minimum total conversion of about 10%. The "Constraint Index" is calculated as follows:

$$\text{Constraint Index} = \frac{\log_{10}(\text{fraction of hexane remaining})}{\log_{10}(\text{fraction of 3-methylpentane remaining})}$$

The Constraint Index approximates the ratio of the cracking rate constants for the two hydrocarbons. Zeolites suitable for the present invention are those having a Constraint Index of at least 2 and up to 12. Constraint Index (CI) values for some typical zeolites including those which are useful herein are:

| Zeolite                  | C.I. (At test temperature) |
|--------------------------|----------------------------|
| ZSM-4                    | 0.5 (316° C.)              |
| ZSM-5                    | 6-8.3 (371° C.-316° C.)    |
| ZSM-11                   | 5-8.7 (371° C.-316° C.)    |
| ZSM-12                   | 2.3 (316° C.)              |
| ZSM-20                   | 0.5 (371° C.)              |
| ZSM-22                   | 7.3 (427° C.)              |
| ZSM-23                   | 9.1 (427° C.)              |
| ZSM-34                   | 50 (371° C.)               |
| ZSM-35                   | 4.5 (454° C.)              |
| ZSM-38                   | 2 (510° C.)                |
| ZSM-48                   | 3.5 (538° C.)              |
| ZSM-50                   | 2.1 (427° C.)              |
| TMA Offrette             | 3.7 (316° C.)              |
| TEA Mordenite            | 0.4 (316° C.)              |
| Clinoptilolite           | 3.4 (510° C.)              |
| Mordenite                | 0.5 (316° C.)              |
| REY                      | 0.4 (316° C.)              |
| Amorphous Silica-alumina | 0.6 (538° C.)              |
| Dealuminized Y           | 0.5 (510° C.)              |
| Erionite                 | 38 (316° C.)               |
| Zeolite Beta             | 0.6-2.0 (316° C.-399° C.)  |

The above-described Constraint Index is an important and even critical definition of those zeolites which are suitable for modification in accordance with the method of this invention. The very nature of this parameter and the recited technique by which it is determined, however, admit of the possibility that a given zeolite can be tested under somewhat different conditions and thereby exhibit different Constraint Indices. Constraint Index seems to vary somewhat with severity of operation (conversion) and the presence or absence of binders. Likewise, other variables such as crystal size of the zeolite, the presence of occluded contaminants, etc., may affect the constraint index. Therefore, it will be appreciated that it may be possible to so select test conditions as to establish more than one value in the range of 1 to 12 for the Constraint Index of a particular zeolite. Such a zeolite exhibits the constrained access as herein defined and is to be regarded as having a Constraint Index in the range of 1 to 12. Also contemplated herein as having a Constraint Index in the range of 1 to 12 and therefore within the scope of the defined novel class of highly siliceous zeolites are those zeolites which, when tested under two or more sets of conditions within the above-specified ranges of temperature and conversion, produce a value of the Constraint Index slightly less than 1, e.g., 0.9, or somewhat greater than 12, e.g., 14 or 15, with at least one other value within the range of 1 to 12. Thus, it should be understood that the Constraint Index value used herein is an inclusive rather than an exclusive value. That is, a crystalline zeolite

when identified by any combination of conditions within the testing definition set forth herein as having a Constraint Index in the range of 1 to 12 is intended to be included in the instant novel zeolite definition whether or not the same identical zeolite, when tested under other of the defined conditions, may give a Constraint Index value somewhat outside the range of 1 to 12.

The class of zeolites defined herein as suitable for undergoing surface modification is exemplified by ZSM-5, ZSM-11, ZSM-12, ZSM-22, ZSM-23, ZSM-35, ZSM-38, ZSM-48, and other similar materials.

ZSM-5 which is especially preferred is described in greater detail in U.S. Pat. No. 3,702,886 and U.S. Pat. No. Re. 29,948. The entire descriptions contained within those patents, particularly the X-ray diffraction pattern of therein disclosed ZSM-5, are incorporated herein by reference.

ZSM-11 is described in U.S. Pat. No. 3,709,979. That description, and in particular the X-ray diffraction pattern of said ZSM-11, is incorporated herein by reference.

ZSM-12 is described in U.S. Pat. No. 3,832,449. That description, and in particular the X-ray diffraction pattern disclosed therein, is incorporated herein by reference.

ZSM-22 is described in U.S. patent application Ser. No. 373,451 filed Apr. 30, 1982, and now pending. The entire description thereof is incorporated herein by reference.

ZSM-23 is described in U.S. Pat. No. 4,076,842. The entire content thereof, particularly the specification of the X-ray diffraction pattern of the disclosed zeolite, is incorporated herein by reference.

ZSM-35 is described in U.S. Pat. No. 4,016,245. The description of that zeolite, and particularly the X-ray diffraction pattern thereof, is incorporated herein by reference.

ZSM-38 is more particularly described in U.S. Pat. No. 4,046,859. The description of that zeolite, and particularly the specified X-ray diffraction pattern thereof, is incorporated herein by reference.

ZSM-48 is more particularly described in U.S. Pat. No. 4,375,573. Such a description includes the x-ray diffraction pattern for ZSM-48.

It is to be understood that by incorporating by reference the foregoing patents and patent applications to describe examples of specific members of the novel class with greater particularity, it is intended that identification of the therein disclosed crystalline zeolites be resolved on the basis of their respective X-ray diffraction patterns. As discussed above, the present invention contemplates utilization of such catalysts wherein the mole ratio of silica to alumina is essentially unbounded. The incorporation of the identified patents and patent applications should therefore not be construed as limiting the disclosed crystalline zeolites to those having the specific silica-alumina mole ratios discussed therein, it now being known that such zeolites may be substantially aluminum-free and yet, having the same crystal structure as the disclosed materials, may be useful or even preferred in some applications. It is the crystal structure, as identified by the X-ray diffraction "fingerprint", which establishes the identity of the specific crystalline zeolite material.

Natural zeolites may sometimes be converted to zeolite structures of the class herein identified by various activation procedures and other treatments such as base

exchange, steaming, alumina extraction and calcination, alone or in combination. Natural minerals which may be so treated include ferrierite, brewsterite, stilbite, dachiardite, epistilbite, heulandite, and clinoptilolite. However, the preferred crystalline zeolites for utilization herein include ZSM-5, ZSM-11, ZSM-12, ZSM-22, ZSM-23, ZSM-35, ZSM-38 and ZSM-48 with the acid or ammonium form such as HZSM-5 or NH<sub>4</sub>/ZSM-5 being particularly preferred.

In a preferred aspect of this invention, the zeolites hereof are selected as those providing among other things a crystal framework density, in the dry hydrogen form, of not less than 1.6 grams per cubic centimeter. It has been found that zeolites which satisfy all three of the discussed criteria are most desired for several reasons. When hydrocarbon products or by-products are catalytically formed, for example, such zeolites tend to maximize the production of gasoline boiling range hydrocarbon products. Therefore, the preferred zeolites useful with respect to this invention are those having a Constraint Index as defined above of about 1 to about 12, a silica to alumina mole ratio of at least about 12 and a dried crystal density of not less than about 1.6 grams per cubic centimeter. The dry density for known structures may be calculated from the number of silicon plus aluminum atoms per 1000 cubic Angstroms, as given, e.g., on Page 19 of the article ZEOLITE STRUCTURE by W. M. Meier. This paper, the entire contents of which are incorporated herein by reference, is included in PROCEEDINGS OF THE CONFERENCE ON MOLECULAR SIEVES, (London, April 1967) published by the Society of Chemical Industry, London, 1968.

When the crystal structure is unknown, the crystal framework density may be determined by classical pycnometer techniques. For example, it may be determined by immersing the dry hydrogen form of the zeolite in an organic solvent which is not sorbed by the crystal. Or, the crystal density may be determined by mercury porosimetry, since mercury will fill the interstices between crystals but will not penetrate the intracrystalline free space.

It is possible that the unusual sustained activity and stability of this special class of zeolites is associated with its high crystal anionic framework density of not less than about 1.6 grams per cubic centimeter. This high density must necessarily be associated with a relatively small amount of free space within the crystal, which might be expected to result in more stable structures. This free space, however, is important as the locus of catalytic activity.

Crystal framework densities of some typical zeolites, including some which are not within the purview of this invention, are:

|                | Void Volume | Framework Density |
|----------------|-------------|-------------------|
| Ferrierite     | 0.28 cc/cc  | 1.76 g/cc         |
| Mordenite      | .28         | 1.7               |
| ZSM-5,11       | .29         | 1.79              |
| ZSM-12         | —           | 1.8               |
| ZSM-23         | —           | 2.0               |
| Dachiardite    | .32         | 1.72              |
| L              | .32         | 1.61              |
| Clinoptilolite | .34         | 1.71              |
| Laumontite     | .34         | 1.77              |
| ZSM-4 (Omega)  | .38         | 1.65              |
| Heulandite     | .39         | 1.69              |
| P              | .41         | 1.57              |

-continued

|           | Void Volume | Framework Density |
|-----------|-------------|-------------------|
| Offretite | .40         | 1.55              |
| Levynite  | .40         | 1.54              |
| Eriomite  | .35         | 1.51              |
| Gmelinite | .44         | 1.46              |
| Chabazite | .47         | 1.45              |
| A         | .5          | 1.3               |
| Y         | .48         | 1.27              |

When synthesized in the alkali metal form, the zeolite is conveniently converted to the hydrogen form, generally by intermediate formation of the ammonium form as a result of ammonium ion exchange and calcination of the ammonium form to yield the hydrogen form. In addition to the hydrogen form, other forms of the zeolite wherein the original alkali metal has been reduced to less than about 1.5 percent by weight may be used.

In the first step of the method herein, the as synthesized zeolite, i.e., one containing the organic template material, is steamed in a known manner to partially or completely decompose the template material and at the same time, to remove framework (zeolitic) aluminum, preferentially aluminum located at the surface of the zeolite. Steaming frequently results in the presence of a carbon residue which can be removed by calcining either immediately following the steaming operation or at some later stage in the method of this invention. Steaming is carried out in accordance with conventional procedures and within conventional limits, none of the latter being particularly critical to the result. Thus, steaming can be carried out for from about 30 minutes to 100 hours at temperature of from about 100° C. to about 600° C. at pressures ranging from subatmospheric to about 2000 p.s.i. The optional calcining step also contemplates known procedures and limits, e.g., temperatures of from about 200° C. to about 600° C. in an inert atmosphere of et.c, for from about 1 minutes to about 48 hours.

Following steaming, the ammonium, alkali metal or hydrogen form of the zeolite is contacted with an aluminum complexing agent, e.g., in accordance with the procedures described in U.S. Pat. No. 4,093,560, the contents of which are incorporated by reference herein. According to U.S. Pat. No. 4,093,560, a slurry of zeolite in the ammonium or alkali metal form is contacted with an aqueous solution of an ammonium or alkali metal salt which, upon acidification, yields an anion which complexes with zeolitic aluminum. The amount of zeolite contained in such slurry will generally be between about 5 and about 60 weight percent. The concentration of the applicable salt solution is usually between about 10 and about 50 weight percent. Suitable salts include the alkali metal and ammonium salts of ethylene diaminetetraacetic acid, such as disodium dihydrogen dethylenediaminetetraacetate and diammonium dihydrogen ethylenediaminetetraacetate; fluoride, such as sodium or ammonium fluoride; carboxylic and polycarboxylic acid salts, such as ammonium acid citrate; mixtures of such complexing agents, etc., including a complexing resin containing an aminodiacetate functional group.

The water soluble acid which is added to the zeolite-containing slurry may be inorganic or organic and of such concentration that the controlled addition thereto does not serve to reduce the pH thereof to below a point where the crystallinity of some zeolites would be ad-

versely affected, i.e., to a pH of below about 3. It is essential that the acid employed be stronger than ethylenediaminetetraacetic acid and thus have a first ionization constant greater than  $10^{-2}$ .

Typical inorganic acids which can be employed include mineral acids such as hydrochloric, sulfuric, nitric and phosphoric acids, peroxydisulfonic acid, dithionic acid, sulfamic acid, peroxymonosulfuric acid, amidodisulfonic acid, nitrosulfonic acid, chlorosulfuric acid, pyrosulfuric acid, and nitrous acid. Representative organic acids which may be used include formic acid, trichloroacetic acid and trifluoroacetic acid.

The concentration of added acid should be such as not to lower the pH of the reaction mixture to an undesirably low level which could affect the crystallinity of the zeolite undergoing treatment. The acidity which the zeolite can tolerate will depend, at least in part, upon the silica/alumina ratio of the starting material. Generally, the pH in the reaction mixture should be greater than about 4 and preferably greater than about 4.5 where the silica/alumina ratio of the starting material is greater than about 2 but less than about 3. When the silica/alumina ratio of the starting material is greater than about 3 but less than about 6, the pH of the reaction mixture should be greater than about 3.

After the described treatment, the product is water washed free of impurities, preferably with distilled water, until the effluent wash water has a pH within the approximate range of 5 to 8. The crystalline dealuminized products obtained by the method of this invention have substantially the same crystallographic structure as that of the starting aluminosilicate zeolite but with increased silica/alumina ratios.

Various other complexing agents, can also be used provided that they form stable chelates with aluminum. In the case of complexing agent which is intended to form soluble complexes or chelates for ease of removal aluminum from the aluminosilicate, the complexing agent should form a stable complex or chelated aluminum which is soluble in the medium, e.g., water in which the complexing is carried out. For a comprehensive review of complexing agents, see "Organic Sequestering Agents" by Stanley Chaberek and Arthur E. Martell, published by John Wiley and Sons, Inc. New York (1959) and an article entitled "Chelation" by Harold F. Walton, Scientific American, June 1953, 68-76, both of which are incorporated herein by reference.

The modified zeolite of the present invention is useful as a catalyst component for a variety of organic, e.g. hydrocarbon, compound conversion processes. Such conversion processes include, as non-limiting examples, cracking hydrocarbons with reaction conditions including a temperature of from about 300° C. to about 700° C., a pressure of from about 0.1 atmosphere (bar) to about 30 atmospheres and a weight hourly space velocity of from about 0.1 to about 20; dehydrogenating hydrocarbon compounds with reaction conditions including a temperature of from about 300° C. to about 700° C., a pressure of from about 0.1 atmosphere to about 10 atmospheres and a weight hourly space velocity of from about 0.1 to about 20; converting paraffins to aromatics with reaction conditions including a temperature of from about 100° C. to about 700° C., a pressure of from about 0.1 atmosphere to about 60 atmospheres, a weight hourly space velocity of from about 0.5 to about 400 and a hydrogen/hydrocarbon mole ratio of from about 0 to about 20; converting olefins to aromat-

ics, e.g. benzene, toluene and xylenes, with reaction conditions including a temperature of from about 100° C. to about 700° C., a pressure of from about 0.1 atmosphere to about 60 atmospheres, a weight hourly space velocity of from about 0.5 to about 400 and a hydrogen/hydrocarbon mole ratio of from about 0 to about 20; converting alcohols, e.g. methanol, or ethers, e.g. dimethylether, or mixtures thereof to hydrocarbons including aromatics with reaction conditions including a temperature of from about 275° C. to about 600° C., a pressure of from about 0.5 atmosphere to about 50 atmospheres and a liquid hourly space velocity of from about 0.5 to about 100; isomerizing xylene feedstock components with reaction conditions including a temperature of from about 230° C. to about 510° C., a pressure of from about 3 atmospheres to about 35 atmospheres, a weight hourly space velocity of from about 0.1 to about 200 and a hydrogen/hydrocarbon mole ratio of from about 0 to about 100; disproportionating toluene with reaction conditions including a temperature of from about 200° C. to about 760° C., a pressure of from about atmospheric to about 60 atmospheres and a weight hourly space velocity of from about 0.08 to about 20; alkylating aromatic hydrocarbons, e.g. benzene and alkylbenzenes, in the presence of an alkylating agent, e.g. olefins, formaldehyde, alkyl halides and alcohols, with reaction conditions including a temperature of from about 340° C. to about 500° C., a pressure of from about atmospheric to about 200 atmospheres, a weight hourly space velocity of from about 2 to about 2000 and an aromatic hydrocarbon/alkylating agent mole ratio of from about 1/1 to about 20/1; and transalkylating aromatic hydrocarbons in the presence of polyalkylaromatic hydrocarbons with reaction conditions including a temperature of from about 340° C. to about 500° C., a pressure of from about atmospheric to about 200 atmospheres, a weight hourly space velocity of from about 10 to about 1000 and an aromatic hydrocarbon/polyalkylaromatic hydrocarbon mole ratio of from about 1/1 to about 16/1.

As previously indicated, the modified crystalline silicate zeolite of this invention is especially advantageous for use in catalyzing the conversion of lower olefins to provide high viscosity lubes, an example of which is given below. Suitable lower olefins generally include C<sub>2</sub> to C<sub>8</sub> olefins with propylene and butylene or mixtures thereof being preferred. However, higher olefins can be used but for greater cost effectiveness the inexpensive lower olefins are preferably.

In the examples which follow, Examples 1 and 2 illustrate modification of an as synthesized zeolite employing the step of contacting the zeolite with dealuminizing agent but omitting steaming. Example 3 is illustrative of the catalyst modifying process herein which includes steps of steaming and contacting with dealuminizing agent and Example 4 compares the results of oligomerizing a lower olefin, i.e., propylene, employing the foregoing modified zeolites as well as unsteamed and steamed non-modified zeolite.

#### EXAMPLE 1

8 g of 1/25" NH<sub>4</sub>ZSM-5 silica extrudate was added to 300 ml aqueous solution containing 0.25 g Na<sub>2</sub>EDTA. The reaction mixture was digested at about 100° C. for 4 hrs. The product was cooled, washed, exchanged with 1N NH<sub>4</sub>Cl and calcined to provide surface-modified ZSM-5. Analysis of the starting zeolite and the EDTA-modified zeolite is shown in Table 1.

4,876,411

11

TABLE 1

|                                      | Starting NH <sub>4</sub> ZSM-5 | EDTA-modified ZSM-5 |
|--------------------------------------|--------------------------------|---------------------|
| Silica/alumina ratio                 | 70/1                           | 80/1                |
| Exchange capacity<br>(meq/g zeolite) | 0.46                           | 0.38                |
| Hexane cracking activity             | 160                            | 180                 |

## EXAMPLE 2

16 grams of as-synthesized tetrapropylammonium (TPA) bromide-containing ZSM-5 binder free extrudate of 70/1 silica to alumina ratio was slurried with 0.5 gm disodium ethylene diamine tetraacetic acid (Na<sub>2</sub>EDTA) in 400 ml H<sub>2</sub>O (pH adjusted to 2.5 with 0.2N HCl) for 26 hours at room temperature. Following decantation of the liquid, the catalyst was washed with water, dried at 130° C. and calcined using a stream of 500 cc/min N<sub>2</sub> and 50 cc/min air with temperature increased 1° C./min to 525° C. and held 10 hours. The calcined catalyst was exchanged with 1N NH<sub>4</sub>NO<sub>3</sub> soln and another Na<sub>2</sub>EDTA extraction was carried out for 8 hours. The resulting catalyst was washed with deionized water and calcined as above. Ammonia ion-exchange capacity was measured by TPAD, MEQ/gm Cat=0.42, SiO<sub>2</sub>/Al<sub>2</sub>O<sub>3</sub> about 79.

## EXAMPLE 3

12 grams of as-synthesized TPA 70/1 100% ZSM-5 extrudate was exchanged with 400 ml of 1N NH<sub>4</sub>NO<sub>3</sub> (pH adjusted to about 2 with dilute HNO<sub>3</sub>) to remove surface and excess sodium, then washed, dried, and steamed. Steaming conditions were 810° F., 6.5 h, 100% steam, and 1 atm. Following steaming, the catalyst was exchanged with 500 ml 1N NH<sub>4</sub>NO<sub>3</sub> at room temperature, washed, dried, and calcined. The calcined catalyst was slurried in a solution containing 0.8 g Na<sub>2</sub>EDTA in 400 ml water. The pH of the slurry was adjusted with dilute HNO<sub>3</sub> to about 3 and the mixture was refluxed at about 95° C. for 23 hours. The product was cooled, washed, and exchanged with 600 ml 1N NH<sub>4</sub>NO<sub>3</sub> for 6 hours. The resultant catalyst was washed, dried, and calcined to provide surface-modified ZSM-5. Analysis of the starting zeolite and the surface-modified ZSM-5 is shown in Table 2.

TABLE 2

|                                      | Starting ZSM-5 | Surface-Modified ZSM-5 |
|--------------------------------------|----------------|------------------------|
| Silica/alumina ratio                 | 70/1           | 108                    |
| Exchange capacity<br>(meq/g zeolite) | 0.45           | 0.30                   |

## EXAMPLE 4

Propylene was oligomerized over the catalyst of Examples 1, 2 and 3 at 440° F. and 400 psig in a stainless steel micro-unit with a  $\frac{5}{8}$ " inner diameter containing 15 cc of catalyst. For purposes of comparison, oligomer-

12

ization was also carried out with (unmodified) HZSM-5 alumina extrudate. The data are set forth in Table 3 below. The last two columns of Table 3 show data collected over unsteamed and steamed (900° F. for 6 hrs.) HZSM-5 alumina extrudate.

TABLE 3

|                      | HZSM-5 Extrudate |           |           |                                                                              |     |    |
|----------------------|------------------|-----------|-----------|------------------------------------------------------------------------------|-----|----|
|                      | Modified ZSM-5   |           |           | Un-Steamed<br>70/1<br>SiO <sub>2</sub> /Al <sub>2</sub> O <sub>3</sub>       |     |    |
|                      | Example 1        | Example 2 | Example 3 | Steamed<br>900° F./6 hrs<br>SiO <sub>2</sub> /Al <sub>2</sub> O <sub>3</sub> |     |    |
| LHSV                 | 0.2              | 0.2       | 0.2       | 0.5                                                                          | 1.0 | —  |
| TOS, days<br>650° F. | 11               | 15        | 6         | 2                                                                            | 6   | —  |
| lube<br>wt. %        | 31               | 29        | 35        | 30                                                                           | 22  | 18 |
| VI                   | 79               | 77        | 75        | 90                                                                           | 95  | 73 |
|                      |                  |           |           |                                                                              |     | 9  |
|                      |                  |           |           |                                                                              |     | 43 |

From Table 3, it can be seen that ~30 wt. % lube yields with 5 to 79 and 90 VI were obtained with the catalyst of Examples 1, 2, and 3 compared with unmodified, unsteamed catalyst which gave an 18 wt. % lube yield with 73 VI. Unmodified, steamed HZSM-5 yielded 10 wt. % lube with 43 VI, compared to the catalyst of Example 3 which gave 22 wt. % lube yield with 95 VI. These data further establish the criticality of carrying out steaming prior to subjecting the as synthesized zeolite to being contacted with the dealuminizing agent. Thus, very substantial VI increases were obtained with the catalyst of Example 3 compared with those of Examples 1 and 2.

What is claimed is:

1. A process for the production of high viscosity index lubricating oils in high yields from lower olefin comprising contacting said olefin over a modified crystalline aluminosilicate ZSM-5 zeolite catalyst resulting from a method which comprises:
  - (a) steaming an synthesized crystalline aluminosilicate ZSM-5 zeolite containing organic template material to decompose at least a portion of said template material and to extract zeolitic aluminum; and
  - (b) contacting the ZSM-5 zeolite resulting from step (a) in the ammonium, alkali metal or hydrogen form with a dealuminizing agent which forms a water-soluble complex with aluminum to remove a further quantity of zeolitic aluminum therefrom.
2. The process of claim 1 wherein the olefin is selected from the group consisting of propylene and butylene.
3. The process of claim 1 wherein the modified zeolite resulting from step (b) is calcined to provide the hydrogen form of the zeolite.
4. The process of claim 1 wherein in step (b), the steamed zeolite in the ammonium, alkali metal or hydrogen form is slurried with an aqueous solution of an ammonium or alkali metal salt which upon acidification yields an anion which complexes with aluminum, a water-soluble acid thereafter being added to said aqueous slurry to provide the dealuminizing agent.
5. The process of claim 4 wherein said acid is a mineral acid.
6. The process of claim 5 wherein said mineral acid is hydrochloric acid.
7. The process of claim 4 wherein said salt is an ammonium or alkali metal ethylenediaminetetraacetate.
8. The process of claim 4 wherein said salt is disodium dihydrogen ethylenediaminetetraacetate.
9. The method of claim 4 wherein said salt is diammonium dihydrogen ethylenediaminetetraacetate.

\* \* \* \* \*